

Nov. 15, 1955

G. S. HOOPER

2,723,900

SPINNING OF ACRYLONITRILE POLYMERS

Filed Dec. 3, 1952

2 Sheets-Sheet 1



Nov. 15, 1955

G. S. HOOPER

2,723,900

## SPINNING OF ACRYLONITRILE POLYMERS

Filed Dec. 3, 1952

2 Sheets-Sheet 2

INVENTOR  
GILMAN S. HOOPER

BY Philip J. Canepa  
ATTORNEY

# United States Patent Office

2,723,900

Patented Nov. 15, 1955

1

2,723,900

## SPINNING OF ACRYLONITRILE POLYMERS

Gilman S. Hooper, Bay Village, Ohio, assignor to Industrial Rayon Corporation, Cleveland, Ohio, a corporation of Delaware

Application December 3, 1952, Serial No. 323,757

22 Claims. (Cl. 18—54)

This invention relates to an improved method of producing fibers, threads, yarns, tows and the like (hereinafter referred to as fibers) by wet-spinning water-containing ethylene carbonate spinning solutions of acrylonitrile polymers and copolymers in an aqueous coagulating bath. More particularly, it is concerned with a method for treating and processing the wet-spun freshly coagulated fiber.

The wet-spinning or wet-forming of ethylene carbonate-solvent type spinning solutions of acrylonitrile polymers was first described in the copending U. S. application of John M. Terpay, Serial No. 245,697, filed September 8, 1951, issued August 30, 1955, as U. S. Patent No. 2,716,586. The invention described in that application is concerned with those conditions of the spinning solution and of the coagulating liquid bath which are necessary to achieve successful aqueous-bath spinning. Among other factors, it was established by that invention that ethylene carbonate-solvent spinning solutions of acrylonitrile polymers and copolymers, containing at least about 80% by weight of acrylonitrile in the polymer molecule, could be extruded successfully into aqueous baths if certain amounts of water were incorporated in the ethylene carbonate spinning solution and if the aqueous coagulating liquid contained certain concentrations of ethylene carbonate.

The water-bath spinning process of the Terpay discovery (supra) provides a very simple system in which the only materials involved in the processing in addition to the polymer are water and ethylene carbonate. Furthermore, this process lends itself to a variety of aftertreating and regenerating methods and techniques. However, some difficulty is encountered which is believed largely due to the peculiar nature of the polymer solvent employed and the conditions under which it is used. For example, the solvent ethylene carbonate is an ester which is highly sensitive to water thus requiring very careful control of the aqueous regenerating conditions in order to achieve the desired fiber properties. Moreover, this ester is quite susceptible to hydrolysis particularly when in contact with water for prolonged washing periods and especially at elevated temperatures. Accordingly, the fiber treatment process of this invention is directed particularly to those conditions under which the freshly coagulated fibers, made available by the Terpay discovery (supra), can be regenerated, oriented and water-washed free of the solvent while effecting optimum economy with respect to ethylene carbonate; and while producing fibers of desirably high tensile strength and elongation and of low residual solvent content. Other advantages of the process will become apparent from the subsequent description.

The process in accordance with the present invention is as follows. An ethylene carbonate spinning solution comprising water, in an amount between about 2.5% and 18.5% by weight, and an acrylonitrile polymer or copolymer, containing in the polymer molecule at least about 80% by weight of acrylonitrile, is extruded into an aqueous coagulating liquid comprising water and between

2

about 10% and 50% of ethylene carbonate solvent. The freshly coagulated fiber is withdrawn from the coagulant and is stretched. Some portion or all of the stretching operation is performed in a hot, above 80° C., aqueous liquid having a relatively low ethylene carbonate content, and preferably the fiber is kept in contact with the hot liquid for a short period of time. The hot-stretch liquid referred to contains ethylene carbonate at a concentration less than that of the coagulating liquid and preferably less than about 6% by weight. Advantageously, if desired, the freshly formed fiber may be given a stretch prior to the hot-stretch mentioned. The hot-stretched fiber is then subjected to an aqueous washing treatment which is hereinafter referred to as the "intermediate-wash." The aqueous washing liquid employed for the intermediate-wash contains ethylene carbonate at a concentration which is also less than that of the coagulating liquid but is greater than that of the liquid of the preceding hot-stretch treatment. The intermediate-wash liquid is prepared with part, and preferably all, of the effluent resulting from the hot-stretch treatment. In an analogous manner, part, and preferably all, of the aqueous effluent resulting from the intermediate-wash treatment is used to fortify or "buck-up" the coagulating liquid. In this manner the coagulant is fortified with water to compensate for the ethylene carbonate entering with the extruded spinning solution. The washed fiber resulting from the intermediate-wash treatment is then subjected to another wash treatment which is referred to hereinafter as the "subsequent-wash." At least one of the aqueous liquids, and preferably, the last liquid applied to the fiber for said subsequent-wash treatment is a liquid which is substantially free from ethylene carbonate, e. g. water. Part and preferably all of the effluent resulting from the subsequent-wash, i. e. an aqueous liquid relatively low in ethylene carbonate, is diverted to be used in making up the hot-stretch treating liquid previously described. The resulting completely washed fiber is then in a suitable condition to be dried and collected directly or it may be collected after previously subjecting the fiber to any one or more aftertreatments as desired such as, for example, applying oil finishing agents, heat-relaxing, heat-treating, drying, crimping, cutting, etc.

As mentioned, the spinning solution suitable for successful practice of the process of the present invention is of the type described in the Terpay patent, supra. In addition to the polymer and ethylene carbonate solvent, such spinning solution contains water between about 2.5% and about 18.5% by weight, particular advantages being derived at between about 10% and 15%. The polymer-solids content of the spinning solution may be between about 8% and about 30% by weight; superior results being obtained, however, with a solids content between about 12% and 18%. A reliable index of the spinnability of a given water-containing spinning solution of the type described is the "cloud point." The "cloud point" as used herein is expressed as the temperature at which such a spinning solution changes from a cloudy or turbid solution to a clear transparent solution. The "cloud point" of the solution is a factor in determining more suitable combinations of solids, water and solvent in the spinning solution and preferably should not exceed about 70° C.

The coagulating liquid into which the spinning solution is extruded comprises water and ethylene carbonate solvent in an amount between about 10% and 50% by weight, sampled at a point within three inches from the spinneret. Greater advantages are derived when employing coagulating liquids containing between about 20% and 38% ethylene carbonate solvent by weight. It is found preferable to employ coagulating liquids consisting essentially of water and ethylene carbonate. The coagu-

lating liquid is advantageously maintained at a temperature between about 40° C. and about 90° C.

The fiber resulting from the extrusion of the spinning solution into the coagulating liquid is withdrawn from the coagulating liquid and before being subjected to the aqueous hot-stretch treatment may, if desired, be given a preliminary orientation by stretching so as to increase the total over-all stretch. Preliminary stretches of at least about 150% or more of the original length of the fiber are found highly advantageous.

As indicated the hot-stretch treatment of the fiber is performed in a hot aqueous liquid which has a relatively low ethylene carbonate content and is maintained at a temperature above about 80° C., optimum hot-stretching conditions being achieved at temperatures above about 95° C. and preferably at the boil. Advantageously, the fiber is hot-stretched to a length 150% of its original length or greater if desired. In other words, a given length of fiber, that is, one meter, would be stretched to a total length of one and one-half meters or 150% of (1½ times) its original length.

The primary function of the hot-stretch treatment as employed in the present process is not as much concerned with any washing action as it is to achieve the desired amount of orientation without either deleteriously affecting the character of the fiber or adversely affecting the efficiency of the process. It is found that particularly advantageous results are derived when the amount of fiber-washing action of the hot-stretch liquid is minimized. It is recognized, however, that some incidental washing will of necessity occur. In general, these stretching conditions are achieved by employing an aqueous hot-stretch liquid having a relatively low, yet a carefully controlled, ethylene carbonate content and also by minimizing advantageously the length of time both the fiber and the liquid are held at the elevated stretch temperatures prescribed.

Thus, for example, it is found that an aqueous hot-stretch liquid containing too much ethylene carbonate is detrimental to the process. Among other effects, it is found that there is under such conditions excessive hydrolysis of the solvent at the temperature of the hot-stretch treatment. Hence, in practicing this invention, it is found advantageous to employ aqueous hot-stretch liquids containing between about at least 0.5% and preferably less than 10% by weight of ethylene carbonate. Greater advantages, however, are derived when the ethylene carbonate concentration is maintained between about 1% and 6% by weight.

As indicated, it is also advantageous to minimize the length of time both the fiber and the aqueous treating liquid are held at the elevated hot-stretch temperatures. In general, the minimum time of contact of the fiber with the hot aqueous liquid is that time which is necessary to achieve the desired orientation, or more specifically, the minimum time required to heat the fiber to the optimum condition for stretching. This interval of time may vary depending upon the hot-stretch temperature employed and the denier of the yarn or tow undergoing hot-stretch orientation. Preferably, the time of contact may be between about 0.2 to 2.5 seconds and most advantageously, less than one second. Thus, by minimizing the contact time of the fiber and liquid in the heated stretch zone, the amount of washing action is advantageously reduced to a minimum and greater benefits are derived.

Although various methods and techniques are available for achieving these desirable conditions, the following technique is found quite advantageous for simultaneously controlling the ethylene carbonate concentration of the hot-stretch liquid, minimizing the amount of washing action on the fiber and also minimizing the contact time of both the fiber and the liquid to the elevated temperatures. Thus, for example, the hot-stretch treatment may be performed in a narrow, shallow trough

or tube equipped with heating elements and designed to contain the minimum operable volume of hot-stretch liquid. The liquid may be passed through the heated trough at a very rapid rate so as to maintain a positive control of the ethylene carbonate content of the liquid in the fiber-liquid contact zone. The liquid is thereby quickly heated to the requisite temperature. With advantage, the liquid leaving the heated effective zone of the trough is thereafter rapidly cooled. Thus, the hot-stretch liquid is exposed to an elevated temperature for only a small interval of time.

In practicing the process of this invention, it is found advantageous to maintain the residual ethylene carbonate content of the fiber entering the hot-stretch liquid at 15 between about 75% and 200% by weight, based on the weight of the dried fiber, while maintaining the residual ethylene carbonate content of the fiber leaving the hot-stretch liquid at about 50% to 150%. Particular advantages are derived, however, when the fiber entering the hot-stretch liquid contains between about 125% and 200% of residual ethylene carbonate.

In the intermediate-wash treatment which follows the hot-stretch treatment just described, the fiber is subjected to washing, in one or more stages, with an aqueous liquid which has a greater concentration of ethylene carbonate than the aqueous hot-stretch liquid and preferably, at least about 5% by weight less than that of the coagulating liquid. Thus, for example, if the coagulant contains 30% ethylene carbonate the intermediate-wash 20 would contain less than 25% and the hot-stretch liquid less than about 10% and preferably less than about 6%. Greater advantages, however, are derived when the ethylene carbonate content of the intermediate-wash liquid is maintained less than about 15% by weight. 35 The temperature of the intermediate-wash liquid is advantageously not greater than 60° C. and preferably, between about 40° and 60° C.

Particular benefits are derived when the duration of the intermediate-wash treatment is such that the resulting washed fiber upon withdrawal from the wash liquid 40 described contains between about 25% and 75% by weight of residual ethylene carbonate solvent.

In accordance with the present process, this intermediate-wash liquid is prepared with at least a portion, 45 and preferably all, of the effluent resulting from the hot-stretch treatment of the preceding step. The intermediate-wash liquid thus prepared is applied to the running fiber so that it flows countercurrent to the direction of travel of the fiber. Where a plurality of washing stages are employed to perform this step, the freshly 50 prepared intermediate-wash liquid is first introduced into the last of such series of stages and flows to the first of such stages.

Analogously, as mentioned, part and preferably all, of 55 the effluent resulting from the intermediate-wash treatment is diverted to be incorporated into the coagulating liquid for the purpose of fortifying or bucking-up the latter to thereby maintain the coagulant at the desired water-to-ethylene carbonate ratio. In practicing this invention it is found that this buck-up effluent should contain no more than about 8½ parts by weight of water to each part by weight of spin solution extruded. Special 60 benefits are derived when this effluent contains at least about 5 parts by weight of water to each part by weight of dry fiber extruded. It is highly advantageous for conditions to be such that the maintenance of the coagulating liquid at the desired water-to-ethylene carbonate ratio requires the ratio of water-to-dry fiber in the buck-up effluent from the intermediate-wash to be 65 between about 7 and about 26 parts by weight of water to each part by weight of dry fiber extruded. In general, the required ratio of water-to-solvent diminishes as the relative proportion of ethylene carbonate in the spinning solution decreases or that in the coagulating liquid increases within the general limits previously described 70 75

therefor. Under these conditions, relatively smaller quantities of buck-up effluent are required to compensate for the ethylene carbonate accumulation caused by the extrusion of the spinning solution into the coagulant.

Whatever portion of the aqueous effluent resulting from the intermediate-wash treatment is not diverted as buck-up for the coagulating liquid may, if desired, be by-passed directly to the solvent recovery system, along with the effluent coming from the coagulating bath. These effluents are then subjected to a suitable recovery treatment to separate the ethylene carbonate solvent from the water. The recovered solvent, after being further purified, is suitable for appropriate re-use in the preparation of spinning solution.

The washed fiber, after withdrawal from the intermediate-wash, is subjected to the subsequent-wash treatment of the present process. This washing step also may be performed in one or more stages and is effective in removing substantially all of the remaining quantities of residual solvent present in the fiber. As mentioned, at least one of the last aqueous liquids applied to the fiber for the subsequent-wash treatment is a liquid which is substantially free from ethylene carbonate, e. g. water. Although higher temperatures may be employed if desired, the temperature of the subsequent-wash liquid is advantageously not greater than about 60° C. and preferably, between about 40° and 60° C.

At least a portion and preferably all of the effluent resulting from the subsequent-wash treatment just described is used to prepare the liquid for the hot-stretch treatment. The subsequent-wash effluent being diverted to the hot-stretch liquid is maintained at a relatively low concentration of ethylene carbonate, not greater than about 6% by weight and preferably, between about 1% and 3%.

The duration of the subsequent-wash treatment may be controlled so as to wash the fiber substantially all of the residual solvent or, if desired, only part thereof. If desired, in connection with staple production, incompletely washed fiber may be crimped and cut into staple and part of the subsequent-wash treatment may be performed on the fiber in staple form. The present process is capable of producing, commercially and efficiently, a washed fiber containing less than about 3% by weight of residual solvent and if desired as low as 0.5% or less. Upon withdrawal from the subsequent-wash the washed fiber ordinarily contains about 275% to 325% residual water. The finally washed fiber thus produced is in condition suitable to be dried, aftertreated and collected as desired.

Advantageously, all of the water present in the aqueous processing system above described (with the exception of the water contained in the spinning solution), i. e. the water present in the coagulant, hot-stretch, intermediate-wash and subsequent-wash liquids, is introduced as pure water substantially exclusively at one step of the process, namely, at the subsequent-wash treatment. If desired, various amounts, and preferably small amounts, of water may also be introduced at any of the aqueous treatments mentioned, in order to make adjustments in the various ethylene carbonate-water ratios employed for the particular treating liquids concerned. It is particularly advantageous to introduce no more than about 8½ parts by weight of over-all water for each part by weight of spinning solution extruded. It is also advantageous when at least about 6 parts by weight of water is admitted to the subsequent-wash to each part by weight of dry fiber produced. Further, the greatest benefits are derived and the process conducted with optimum result under such conditions that between about 8 and about 27 parts by weight of water is required to be admitted to the subsequent wash to each part of dry fiber produced without any other source of water save that contained in the spinning solution. Especial benefits are derived when the present process is performed on a completely continuous basis, i. e. continuous fiber treatment and with continuous liquid

flows from one liquid treatment step to the next as previously described and as more fully illustrated herein-after. However, if desired, the fiber treatment can be performed batch-wise on non-continuous lengths and with non-continuous liquid flows.

Suitable apparatus for the practice of the method of the present invention is illustrated in the accompanying drawings:

Figure 1 is a diagrammatic perspective view of an embodiment of the process useful for the continuous manufacture of textile yarns.

Figure 2 represents an embodiment adaptable for the continuous production of heavy denier yarns, tows and the like.

Referring to Figure 1, reference numeral 10 indicates a mass tube through which the spinning solution comprising polymer, solvent and water is conducted to the immersed multiholed spinneret 11 and thereby extruded into an aqueous coagulating bath 12 comprising ethylene carbonate solvent and water contained in trough 13. The resulting freshly formed, multifilament yarn 15, after passing around guide 14, is withdrawn from the coagulating liquid 12 and conducted to and around thread-storage, thread-advancing device 18 and then to positively driven device 19 which is similar to 18 but driven at a greater peripheral speed thereby stretching the thread therebetween. The thread 15 leaving thread-advancing device 19 is hot-stretched by conducting it about spaced guides 20 and 21 immersed in hot aqueous bath 25 contained in a narrow, shallow trough 26 and then around roller guide 23 and onto a pair of positively driven, thread-storage, thread-advancing drums 30 and 31 rotating at a greater peripheral speed than the preceding thread-advancing device 19. The hot-stretch, aqueous bath 25, which is relatively low in ethylene carbonate, is heated to above 80° C. by the heating coils 27, e. g. electrical or steam coils, located in the trough 26.

The resulting hot-stretched thread 15 which is advanced and stored as a helix about the pair of drums 30 and 31 is immersed in the aqueous bath 32 in trough 33 whereby the stored thread is subjected to the intermediate-wash treatment. The intermediate-wash bath 32 is maintained at a temperature between about 40° and 60° C. and is made up with the aqueous effluent resulting from the hot-stretch treatment. Thus, the effluent from the hot-stretch trough 26 is piped to trough 33 in order to replace the intermediate-wash bath 32 and thus "buck-up" the water-to-ethylene carbonate ratio therein. The effluent from the intermediate-wash trough 33 is in turn passed through pipe 16 into the coagulating bath trough 13 in controlled quantities in order to "buck-up" the water ratio in a similar manner and thereby maintain the coagulating bath 12 at the desired composition.

The washed thread 15 leaving the thread-advancing drums 30 and 31 is then passed to and about another pair of thread-advancing drums 36 and 37 driven at about the same peripheral speed as the preceding drums 30 and 31. The pair of drums 36 and 37 are tilted upwardly in the direction of thread-advance so that any treating liquid applied thereto flows countercurrently to the direction of thread-advance and towards the thread-inlet end of the thread-advancing drums. Water 35 is applied to the helically stored thread by means of tube 34 positioned at the thread-discharge end of the thread-advancing drums. The resulting wash water discharged from the thread-advancing drums 36 and 37 is collected in trough 39 as subsequent-wash effluent 38 and contains a relatively low amount of ethylene carbonate. Effluent 38 is piped to the hot-stretch trough 27 by means of pipe 40 so as to maintain the hot-stretch bath 25 at the low ethylene carbonate concentration desired.

The finally washed thread 15 leaving drums 36 and 37 is conducted to a third pair of thread-advancing drums 41 and 42 which are internally heated by any suitable means, e. g. electrical, steam, etc., so as to dry the thread

helically stored thereon. The dried thread leaving the heated drums is then passed through guide 43 and collected on bobbin 45 by means of cap-twisting device 44. The effluent from the coagulating bath 12, containing a greater concentration of ethylene carbonate than the other aqueous treating liquids described, is diverted by pipe 46 to solvent recovery system 47 wherein ethylene carbonate 48 is separated from the water. The recovered ethylene carbonate may be recycled for making the spinning solution.

Referring to Figure 2, reference numeral 59 designates a spinning solution preparation and storage system from which the water-containing spinning solution is passed through (one or more) mass tube 51 to be extruded through (one or more) multiholed spinneret 52 into aqueous coagulating liquid 53, in trough 54. The resulting freshly formed multifilament high-denier yarn 55 or tow, as the case may be, is withdrawn from coagulating liquid 53 about roller guide 56. The yarn, flattened in the form of a thin ribbon, is passed around a set of three yarn-gripping drums 59 positively driven at a predetermined peripheral speed and then around another set of drums 60 similar to the first set but driven at a greater peripheral speed so as to impart a stretch to the yarn between said sets of drums. The yarn 55 from the drums 60 is subjected to the hot-stretch treatment by passing it rapidly through the hot aqueous liquid 65 around spaced guides 63 and 64 in trough 66 and then looped once around each of a pair of drums 70 and succeeding pairs of drums 74, 78, 83, 87 and 91 all of which are positively driven at the same greater peripheral speed than the preceding set of drums 60 so as to hot-stretch the yarn between drums 60 and 70. The hot aqueous liquid 65 is maintained at a temperature above about 80° C. by suitable heating means 62.

The hot-stretched yarn 55 is then subjected to the intermediate-wash treatment which is performed in six stages. The yarn is looped once, as mentioned, around each of six pairs of drums 70, 74, 78, 83, 87 and 91 in succession, the lower of each pair of drums passing through corresponding aqueous washing liquids 71, 75, 79, 84, 88 and 92 contained in troughs 72, 76, 80, 85, 89, and 93 respectively. The yarn from the drums 78 is conducted to drums 83 by first passing it over roller guides 82 and 82A. The yarn moving from the first pair of drums 70 and ultimately to the last pair of drums 91 travels countercurrently to the flow of the corresponding washing liquids while proceeding from trough to trough. Thus, the effluents 90, 86, 81, 77 and 73 from each of the series of intermediate-wash stages flow to the next preceding stage countercurrently to the direction of the yarn.

The aqueous washing liquid 92 present in the last of the series of intermediate-wash stages is made-up with, and replenished by, effluent 94 which is relatively low in ethylene carbonate content and which comes from the preceding hot-stretch treatment of the yarn. The hot effluent 94 after leaving trough 66 is passed through a heat exchanger 95 to be cooled to between 40° and 60° C. before being used as the intermediate-wash liquid 92. Part of effluent 81 coming from the intermediate-wash liquid 84 may, if desired, be by-passed as effluent 68 to the multiport valve 67 and thence as coagulating liquid influent 57 to coagulating liquid 53 while the balance of effluent 81 proceeds to the remaining intermediate-wash stages in order to replenish and replace wash liquids 79, 75 and 71 in succession and resulting finally in effluent 69 leaving trough 72 which may likewise be diverted to valve 67 and thence as coagulating liquid influent 57 to coagulating liquid 53. If desired, however, effluent 69 may be diverted directly through solvent recovery inlet feed 110 to be reclaimed in the solvent recovery system 112. Preferably, the coagulating liquid 53 is bucked-up solely by effluent 69 from the intermediate-wash and no portion of effluent 68 from the stage of the intermediate-

wash in trough 85 is used for this purpose. Coagulating liquid influent 57 from valve 67 which is composed of either effluent 69 or effluent 68 (which is a portion of effluent 81), or both if desired, has a lesser concentration of ethylene carbonate solvent than coagulating liquid 53 so as to be useful for purposes of fortifying the coagulating liquid 53. In the instance when a portion of effluent 81 is diverted as effluent 68 to buck-up coagulating liquid 53 through influent 57, the remainder of the effluent 81 picks up more ethylene carbonate from the yarn stored on drums 78, 74, and 70 and the resulting effluent 69 may contain such a concentration of ethylene carbonate as to be useless for purposes of fortifying coagulating liquid 53. In such case, as mentioned, effluent 69 is diverted directly to the solvent recovery system 112 through inlet 110.

The yarn leaving drums 91, while still in the form of a thin flat ribbon, is then subjected to the subsequent-wash treatment which is performed in three stages. The yarn is looped once around each of three pairs of drums 97, 101 and 105 in succession, the lower of each pair of drums passing through corresponding aqueous wash liquids 98, 102, and 106 contained in troughs 99, 103, and 107 respectively. These aqueous wash liquids are maintained at a temperature between about 40° and 60° C. and originate from water 114 which is freshly introduced into trough 107 at the last stage of the subsequent-wash treatment. The resulting wash-liquid 106 flows from trough 107 in a direction counter to the direction of yarn travel through troughs 103 and 99 as stage effluents 104 and 100 to successively replace and replenish aqueous-wash liquids 102 and 98. Effluent 96 from the subsequent-wash treatment is passed through heat exchanger 95 to be heated by hot effluent 94 coming from the hot-stretch treatment and is thence used to replace and replenish the aqueous liquid 65 in the hot-stretch treatment.

The resulting yarn from the subsequent-wash treatment may be treated with oleaginous finishing agents, antistatic agents, etc., as desired either before or after it is conducted to the internally heated pair of drums 108 where it is dried.

Effluent 57 from coagulating liquid 53 is sent to the solvent recovery system 112 through solvent recovery feed inlet 110 along with any effluent such as effluent 69 from the intermediate-wash treatment. In the solvent recovery system 112 substantially pure ethylene carbonate is recovered by any suitable means. The recovered ethylene carbonate 113 is conducted to the spinning solution system 50. If desired, it may first be decolorized and filtered or otherwise treated so as to be suitable for re-use in preparing the spinning solution along with polymer 115 and spinning solution water 116.

The following examples illustrate specific embodiments of the invention although it is to be understood that there is no intention to restrict the invention to these illustrations. In these examples, "parts" and "percent" of materials, unless otherwise defined, means parts and percent by weight.

#### Example I

In the manufacture of 150 denier yarn, a spinning solution comprising 14 parts of polyacrylonitrile having an average molecular weight of about 40,000, 14 parts of de-mineralized water and 72 parts of ethylene carbonate solvent is prepared. The spinning solution has a "cloud point" of about 55° C. and is heated to about 70° C. for extrusion. Using the apparatus of Figure 1, about 1.02 lbs. per hour of this spinning solution is extruded through mass tube 19 and spinneret 11 having 50 holes, each of 0.003 inch diameter, into coagulating liquid 12 contained in trough 13 consisting of about 67 parts of water and 33 parts of ethylene carbonate.

The coagulating liquid 12 is maintained at about 60° C. while the filaments, freshly formed at a rate of about 0.143 lb. of dry fiber per hour, are drawn through the bath for a distance of about 58 inches. The thread 15 is

withdrawn from the bath containing about 150% residual solvent and about 220% residual water and passed over positively driven thread-storage, thread-advancing device 18 being rotated at a peripheral speed of about 9.7 meters per minute. The thread is then passed in air to positively driven device 19, similar to 18 but rotated at a peripheral speed of about 44.6 meters per minute which imparts an initial stretch to the thread of about 460% of its original length.

Thread 15 is then hot stretched by passing it through hot aqueous liquid 25 for a distance of about 12 inches after which it is withdrawn by positively driven drums 30 and 31 being rotated at a peripheral speed of about 71.4 meters per minute so as to cause the fiber to be additionally stretched to about 160% of its length while immersed in hot liquid 25, which has a relatively low ethylene carbonate content. Liquid 25 is composed of the effluent from the subsequent-wash treatment in pipe 40 which contains about 2.0% ethylene carbonate. It is rapidly passed through trough 26, which has cross-sectional dimensions of  $\frac{3}{4}$  inch width and 3 inch depth, at a rate of about 13.1 cc. per minute at the inlet. The immersion time of thread 15 in hot-stretch liquid 25 is between about 0.25 to 0.41 second. The over-all stretch imparted to the thread by initial orientation and by the hot-stretch treatment is about 736% of its original length. Aqueous liquid 25 is maintained at about 100° C. by means of steam coils 27 located at the bottom of trough 26. The residual solvent content of thread 15 upon being withdrawn from the hot-stretch treatment is about 105% and the residual water content about 275%.

The stretched thread 15 is then given the intermediate-wash treatment by immersion in aqueous liquid 32 contained in trough 33 while being helically passed about positively driven thread-storage, thread-advancing drums 30 and 31. The distance of immersion is about 142 feet and the temperature of liquid 32 is maintained at about 60° C. Liquid 32 is made up with the effluent from the hot-stretch treatment which contains about 6.0% ethylene carbonate upon entering trough 33. The effluent from the intermediate-wash treatment, after washing thread 15, contains about 13.0% ethylene carbonate. This effluent is passed to fortify or buck-up coagulating liquid 12 through pipe 16 and contains about 11.4 parts of water to each part of polymer solids extruded through spinneret 11 per hour or about 1.60 parts of water to each part of spinning solution extruded per hour.

From drums 30 and 31 the thread 15 is withdrawn containing about 25% residual solvent and about 290% residual water. The washed thread is helically passed about drums 36 and 37 operated by positive drive at the same peripheral speed as drums 30 and 31 whereon it is given the subsequent-wash with water 35, substantially free from ethylene carbonate, introduced through tube 34. The subsequent-wash treatment is performed at about 60° C. and the distance of immersion of the thread in the wash liquid is about 292 feet. Liquid 38 which collects in trough 39 underneath the drums 36 and 37 is passed through pipe 40 as effluent from the subsequent-wash which, as mentioned, contains about 2.0% ethylene carbonate.

About 12.4 parts of water 35 are admitted in the subsequent-wash liquid to each part of solids extruded through spinneret 11 per hour or about 1.75 parts to each part of spinning solution extruded per hour. About 1.78 lbs. of water 35 is admitted through tube 34 per hour.

Washed thread 15 is withdrawn from the subsequent-wash containing about 0.5% ethylene carbonate as residual solvent and about 300% residual water. It is then passed about steam heated drums 41 and 42 whereon it is dried and heat-treated prior to being collected on bobbin 45 under cap twisting device 44.

The effluent from coagulating liquid 12 is diverted through pipe 46 to recovery system 47 wherein substantially pure ethylene carbonate 48 is recovered from aque-

ous solution. The recovered ethylene carbonate solvent 48 is suitable for re-use on a continuously recycled basis for the preparation of fresh spinning solution.

A colorless white fiber is produced which is dense and free of objectionable voids on microscopic examination. It has a tenacity of about 3.3 grams per denier and an elongation at break of about 18%.

#### Example II

Using the apparatus of Figure 2, a spinning solution comprising 13 parts of acrylonitrile having an average molecular weight of about 45,000, 14 parts of water and 73 parts of ethylene carbonate solvent is prepared in spinning solution system 50. The spinning solution has a "cloud point" of about 50° C.

In order to produce a yarn of about 44,000 denier, about 315 lbs. per hour of this spinning solution are extruded at about 70° C. through twenty mass tubes 51 and spinnerets 52 (each spinneret having 720 holes of 0.003 inch diameter) into coagulating liquid 53 contained in trough 54 consisting of about 30 parts ethylene carbonate solvent and 70 parts water and maintained at a temperature of about 65° C. The rate of extrusion through each spinneret is about 15.75 lbs. of spinning solution per hour. The resulting freshly formed multifilament yarn 55 is withdrawn about roller guide 56 and flattened in the form of a thin ribbon. This ribbon of yarn 55 is passed to the positively driven yarn gripping drums 59 operated at a peripheral speed of 9.7 meters per minute. From drums 59 the yarn 55 is passed to another set of drums 60, similar to 59 but operated at a peripheral speed of 40.7 meters per minute so as to impart an initial stretch to the yarn of about 420% of its original length. At this point the yarn contains about 162% residual solvent and about 210% residual water. From the drums 60 the yarn is passed through hot aqueous liquid 65 around guides 63 and 64 contained in trough 66 which has a cross-sectional height of three inches and a width of ten inches and then looped around drums 70 operated at a peripheral speed of 61.1 meters per minute thereby imparting an additional stretch to yarn 55 of about 150% of its length while the yarn is subjected to the hot-stretch treatment. Liquid 65 is maintained at 100° C. by means of steam coils 62. The immersion distance of yarn 55 in liquid 65 is about 15 inches and the time of immersion is between about 0.375 to 0.53 second. Liquid 65 is composed of the effluent 96 from the subsequent-wash treatment which contains about 1.55% ethylene carbonate upon entry into trough 66. It is passed through trough 66 at a rate of about 1.21 gallons per minute. Effluent 96 is heated by passage through heat exchanger 95 counter-current to effluent 94 from the hot-stretch treatment which is cooled thereby before being used in the intermediate-wash. Effluent 94 from the hot-stretch treatment contains about 5.12% ethylene carbonate.

Upon withdrawal from the hot-stretch treatment, yarn 55 contains about 112% ethylene carbonate as residual solvent and about 270% residual water. After leaving the hot stretch, the total stretch imparted to yarn 55 is about 630% of its original length.

Yarn 55 is then subjected to the six stage intermediate-wash by being looped about drums 70, 74, 78, 83, 87 and 91 (all positively driven at a peripheral speed of 61.1 meters per minute) and passing for a total wash distance of 130 feet in liquids 71, 75, 79, 84, 88 and 92 maintained at a temperature of about 50° C. and contained respectively in troughs 72, 76, 80, 85, 89 and 93. The intermediate-wash liquid moves from stage trough to stage trough as stage effluents 90, 86, 81, 77 and 73 in a direction counter to the progress of yarn 55 through the stages of the intermediate-wash. The intermediate-wash is prepared by incorporating effluent 96 from the hot-stretch treatment (which, as mentioned, contains about 5.12% ethylene carbonate) in trough 93 as liquid 92. From the last stage of the intermediate-wash the liquid washes yarn

55 until it emerges from trough 72, the first stage of the intermediate-wash, as effluent 69 which contains about 11.3% ethylene carbonate. Effluent 69 is diverted through valve 67 to coagulating liquid 53 so as to maintain in proper correlation the solvent and water constituents thereof. Effluent 69 contains about 14.2 parts water per part solid extruded through spinnerets 52 per hour or about 1.84 parts water per part spinning solution extruded.

The yarn leaving drums 91, still in the form of a thin flat ribbon contains about 25% residual solvent and 280% residual water. It is passed through the subsequent-wash treatment by being looped around drums 97, 101 and 105 in succession and subjected for a total wash distance of 320 feet through the subsequent-wash liquids 98, 102 and 106 maintained at about 50° C. and contained in troughs 99, 103 and 107 respectively. The subsequent-wash liquid is composed of water 114 which, when introduced to the final stage of the subsequent-wash in trough 107, is substantially free of ethylene carbonate. Liquid 106, which is composed of water 114 and the ethylene carbonate washed from yarn 55 on drums 103 is passed as stage effluent 104 to make-up liquid 102 in trough 103 which in turn is passed as stage effluent 109 to make-up liquid 98 in trough 99. Effluent 96 from the subsequent-wash treatment comes from the first stage in trough 99 and, as indicated, contains about 1.55% ethylene carbonate. As mentioned, this effluent is passed through heat exchanger 95 before being used to make-up liquid 65 in the hot-stretch treatment. About 613 lbs. per hour of water 114 are admitted to the last stage of the subsequent-wash in trough 107 which represents about 15.0 parts of water to each part of solids extruded through spinnerets 52 per hour or about 1.95 parts of water to each part spinning solution extruded per hour.

Yarn 55 is withdrawn from drums 105 containing about 2% residual solvent and about 290% residual water. The yarn is dried on steam heated drums 108, then crimped, cut to staple and baled ready for shipment.

Effluent 57 from the coagulating liquid is sent to solvent recovery system 112 through solvent recovery inlet feed 110 wherein substantially pure ethylene carbonate solvent 113 is recovered from aqueous solution. Recovered solvent 113 is continuously recycled to spinning solution system 50 for use in preparing fresh spinning solution. The recovered solvent may advantageously be decolorized with activated charcoal and filtered continuously before re-use in the process.

As is apparent, the yarn may be subjected to the wash treatments in any desired form. For example, it may be cut to staple lengths after withdrawal from the hot-stretch treatment and then subjected to the wash treatments in such form. It may be cut to staple after withdrawal from the intermediate-wash before being given the subsequent-wash. Or, the yarn may be cut to staple lengths during any part of the wash treatments, for example, it may be transformed from continuous filament lengths to staple form after a portion of the subsequent-wash treatment has been performed. In such cases, the balance of the wash treatment, particularly with regard to the employment of wash liquids and resulting effluents, is performed on the staple according to the process of the invention. It is preferable, in any instance, to crimp the continuous filament yarn prior to cutting it into staple, however, if desired, the yarn may be crimped while in staple form after completion of the wash treatments. Other desirable treatments, physical or otherwise, may be performed on the yarn during any stage or interval of the wash treatments.

As is apparent from the foregoing description there are a number of modifications of the process which can be practiced without departing from the scope of the invention. Thus, for example, aqueous treating liquids, i. e. water containing varying amounts of ethylene carbonate or pure water, may be introduced at any of the described treating and washing steps for the purpose of adjusting

either the ethylene carbonate content of the traveling thread or yarn, or the ethylene carbonate content of the various aqueous treating liquids. Accordingly, minor amounts may be added for these purposes prior to the hot-stretch treatment or at any point after the hot-stretch treatment.

The ethylene carbonate solvent used in accordance with the process of the present invention, most advantageously, consists of substantially pure ethylene carbonate. However, if desired, relatively small proportions of other compounds, preferably organic compounds, may be included therein provided they do not amount to more than about 5% by weight of the ethylene carbonate present and, further, that they have no otherwise adverse effect upon the efficiency of the process. Glycol compounds, e. g., ethylene glycol, dipropylene glycol, etc. are among the tolerable organic compounds which may be included in the ethylene carbonate solvent, with advantage.

As previously indicated, orientation stretching of the fiber may be performed at a number of stages of the process in addition to the hot-stretch treatment of the present invention. Thus, preliminary orientation may be imparted to the fiber while it is still in the coagulating bath or, if desired, after it leaves the coagulating bath and while in air or in the presence of other aqueous treating liquids. Moreover, if additional orientation is desired after the hot-stretch treatment the finally washed fiber, preferably containing little or no ethylene carbonate, may be stretched in the presence of steam.

Although greater advantages are derived in practicing the process of this invention in a continuous manner from start to finish with continuous flows of treating liquids from step to step, it is apparent that semi-continuous procedures can also be practiced if desired. Thus, for example, if higher extrusion speeds are desired the continuous length of yarn may be interrupted after the hot-stretch treatment and the yarn collected on a bobbin. Thereafter the washing treatments, i. e. the intermediate-wash and the subsequent-wash, may be performed at relatively lower speeds so as to reduce the size of the washing apparatus.

The recycling of the reusable ethylene carbonate is accomplished after subjecting the effluent from the coagulating bath to a recovery treatment. Thus continuous portions of the bath may be subjected to a flash distillation under sub-atmospheric pressure so as to remove most of the water and the residue thereof thereafter fractionated to recover substantially pure ethylene carbonate solvent. The latter is then treated with decolorizing carbon, filtered and recycled directly for use as solvent in the preparation of additional quantities of spinning solution.

The spinning solution "cloud point" value which is referred to herein, and which was previously characterized as an index of good spinnability, is determined in the following manner. A solution containing the desired proportions of polymer, ethylene carbonate and water is heated until a clear, transparent solution is obtained. The resulting solution is then permitted to cool slowly, with stirring, until the first signs of cloudiness appear. The temperature at which this change takes place is termed the "cloud point." When employing solutions having a "cloud point" between about 20° and 70° C., the turbidity or cloudiness in the solution at the "cloud point" temperature is believed to be a precipitation of the polymer from the solution, whereas with solutions which are still clear and non-turbid at about 20° C., the turbidity or cloudiness which appears upon further cooling may be the same precipitation of the polymer component or it may be a "freezing" or crystallization of the solvent component and more likely a combination of both. In determining the "cloud point," it is particularly important that the solution be cooled slowly. Accordingly, when making cloud point determinations, a cooling medium should be employed which is about 5° C. less than the temperature of the solution being cooled.

This invention may be utilized to produce a variety of final thread or yarn products, i. e., threads having deniers as low as 75 to 50 or high-denier strands or tows for staple. Thus the process is found useful in making the high-denier strands, i. e. over 500 denier and up to 5,000 or more and is particularly useful for making tows of between about 40,000 and 1,000,000 denier. Moreover, these products can be produced at low speeds or more advantageously, at higher speeds ranging from 20 meters per minute or higher.

As previously stated, the proportion of acrylonitrile in the polymer molecule should be at least about 80% by weight and more advantageously, at least about 90% by weight. A minor proportion of one or more vinyl compounds can be copolymerized with the acrylonitrile, for example: vinyl esters (vinyl acetate, vinyl formate, vinyl benzoate), vinyl ethers, and vinyl ketones; acrylic acid and its esters and amides; methacrylic acid and its esters, amides, and nitrile; maleic, itaconic, fumaric, crotonic acids and their esters, amides and nitriles; allyl alcohol and its esters and ethers; styrene and nuclear substituted styrenes, e. g. chloro- and dichloro-styrene; halogenated monoethylenic compounds such as vinyl chloride, vinyl fluoride, vinylidene chloride, 1,2-dichloropropene-1, 1,2-dichloro-propene-2, allyl chloride, methallyl chloride, 2-chloro-allyl alcohol, and 1-allyloxy-3-chloro-2-propanol; N-vinyl compounds such as N-vinyl pyrrolidone, N-vinyl succinimide, N-vinyl carbozole, N-tertiary butyl acrylamide, N-tertiary octyl acrylamide; 2- or 4-vinylpyridine; and the like.

The acrylonitrile polymers may be prepared by any suitable polymerization method such as, for example, polymerization with oxygen-yielding catalysts, e. g. benzoyl peroxide, hydrogen peroxide, tertiary butyl hydroperoxide, potassium or ammonium persulfate, etc. Redox polymerization systems employing oxygen-yielding catalysts such as the above in combination with reducing agents such as sodium bisulfite, sodium hydrosulfite, sodium formaldehyde sulfoxylate, etc., may also be used. Generally, after completion of the polymerization reaction, the resulting polymer is washed with water to remove any remaining impurities.

Although polymeric materials of higher molecular weight may be employed, those between 30,000 and 100,000 are preferred. The spinning solutions employed in the process of the present invention may be prepared by various methods. Thus, for example, one may prepare a room-temperature slurry of the polymer, ethylene carbonate and water and thereafter heat the slurry to effect dissolution of the polymer. If desired, the spinning solution may be prepared by first preparing a polymer solution without the water consisting of ethylene carbonate and between about 15% and 25% of the polymer solids; deaerating this solution and then making the final spinning solution by adding the desired quantity of water in the form of a water-ethylene carbonate mixture.

It is to be understood that all matter contained in the foregoing description be interpreted as illustrative merely and in no sense limiting since certain changes may be made in practicing the invention which in no way departs from its scope.

I claim:

1. In the method of making acrylonitrile polymer fibers by extruding into a coagulating liquid comprising water and between about 10% and 50% by weight of ethylene carbonate, a spinning solution comprising ethylene carbonate, water in an amount between about 2.5% and 18.5% by weight, and a polymer of acrylonitrile containing in the polymer molecule at least about 80% by weight of acrylonitrile, the steps comprising, withdrawing the resulting fiber from said coagulating liquid; stretching said fiber in the presence of an aqueous liquid maintained at a temperature above about 80° C., said hot aqueous stretching liquid comprising water and

ethylene carbonate and having a lower concentration of ethylene carbonate than said coagulating liquid; withdrawing said stretched fiber from said hot-stretching liquid; subjecting said fiber to an intermediate-wash treatment with an aqueous liquid comprising water and ethylene carbonate and having a lower concentration of ethylene carbonate than said coagulating liquid but greater than said hot-stretching liquid, said intermediate-wash liquid being prepared by incorporating at least a portion of the effluent resulting from said hot-stretching treatment; diverting at least a portion of the effluent resulting from said intermediate-wash treatment and fortifying said coagulating liquid therewith; subjecting said fiber to a subsequent-wash treatment with an aqueous liquid which is substantially free from ethylene carbonate; diverting at least a portion of the effluent resulting from said subsequent-wash treatment and incorporating the same into the liquid used in said hot-stretch treatment.

2. In the method of making acrylonitrile polymer fibers by extruding into a coagulating liquid comprising water and between about 10% and 50% by weight of ethylene carbonate, a spinning solution comprising ethylene carbonate, water in an amount between about 2.5% and 18.5% by weight, and a polymer of acrylonitrile containing in the polymer molecule at least about 80% by weight of acrylonitrile, the steps comprising, withdrawing the resulting fiber from said coagulating liquid; stretching said fiber in the presence of an aqueous liquid maintained at a temperature above about 80° C., said hot aqueous stretching liquid comprising water and ethylene carbonate and having a lower concentration of ethylene carbonate than said coagulating liquid; withdrawing said stretched fiber from said hot-stretching liquid, subjecting said fiber to an intermediate-wash treatment with an aqueous liquid comprising water and ethylene carbonate, said intermediate-wash liquid having a lower concentration of ethylene carbonate than said coagulating liquid but greater than said hot-stretching liquid, said intermediate-wash liquid being prepared by continuously incorporating at least a portion of the effluent resulting from said hot-stretching treatment; continuously diverting at least a portion of the effluent resulting from said intermediate-wash treatment and continuously fortifying said coagulating liquid therewith; subjecting said fiber to a subsequent-wash treatment with an aqueous liquid which is substantially free from ethylene carbonate; continuously diverting at least a portion of the effluent resulting from said subsequent-wash treatment and incorporating the same in the liquid used in said hot-stretching treatment; drying said washed fiber.

3. In the method of making acrylonitrile polymer fibers by extruding into a coagulating liquid comprising water and between about 10% and 50% by weight of ethylene carbonate, a spinning solution comprising ethylene carbonate, water in an amount between about 2.5% and 18.5% by weight, and a polymer of acrylonitrile containing in the polymer molecule at least about 80% by weight of acrylonitrile, performing in a continuous manner and on a continuous length of fiber the steps comprising, withdrawing the resulting fiber from said coagulating liquid; stretching said fiber to a length at least about 150% of its original length in the presence of an aqueous liquid maintained at a temperature above about 80° C., said hot aqueous stretching liquid comprising water and between about 0.5% and 10% by weight of ethylene carbonate; withdrawing said stretched fiber from said hot-stretching liquid; subjecting said fiber to an intermediate-wash treatment with an aqueous liquid comprising water and ethylene carbonate, and having a lower concentration of ethylene carbonate than said coagulating liquid but greater than said hot-stretching liquid, said intermediate-wash liquid being prepared by continuously incorporating at least a portion of the effluent resulting from said hot-stretching treatment; continuously diverting at

least a portion of the effluent from said intermediate-wash treatment and continuously fortifying said coagulating liquid therewith so as to assist the maintenance of said coagulating liquid at said concentration, said diverted liquid containing less ethylene carbonate than said coagulating liquid; subjecting said fiber to a subsequent-wash treatment with an aqueous liquid which is substantially free from ethylene carbonate; continuously diverting at least a portion of the effluent resulting from said subsequent-wash treatment and incorporating the same in the liquid used in said hot-stretching treatment; drying said washed fiber.

4. A method according to claim 3 wherein the stretched fiber resulting from said hot-stretching treatment contains less than about 175% by weight of ethylene carbonate and the fiber is stretched a total length of at least about 300% of the original length as withdrawn from the coagulating liquid.

5. A method according to claim 3 wherein the portion of the effluent from the intermediate-wash treatment which is continuously diverted to fortify the coagulating liquid contains at least about five parts by weight of water for each part by weight of said acrylonitrile polymer solids extruded into said coagulating liquid.

6. In the method of making acrylonitrile polymer fibers by extruding into a coagulating liquid comprising water and between about 10% and 50% by weight of ethylene carbonate, a spinning solution comprising ethylene carbonate, water in an amount between about 2.5% and 18.5% by weight, and a polymer of acrylonitrile containing in the polymer molecule at least about 80% by weight of acrylonitrile, performing in a continuous manner and on a continuous length of fiber the steps comprising, withdrawing the resulting fiber from said coagulating liquid; orienting said fiber by stretching it to a length at least about 150% of its original length; stretching said fiber again to a length at least about 150% of its length while in the presence of an aqueous liquid maintained at a temperature above about 80° C., said hot aqueous stretching liquid comprising water and between about 0.5% and 10% by weight of ethylene carbonate; withdrawing said stretched fiber from said hot-stretching liquid; subjecting said fiber to an intermediate-wash treatment with an aqueous liquid comprising water and ethylene carbonate and having a lower concentration of ethylene carbonate than said coagulating liquid but greater than said hot-stretching liquid, said intermediate-wash liquid being prepared by continuously incorporating at least a portion of the effluent resulting from said hot-stretching treatment; continuously diverting at least a portion of the effluent from said intermediate-wash treatment and continuously fortifying said coagulating liquid therewith so as to assist the maintenance of said coagulating liquid at said concentration, said diverted liquid containing less ethylene carbonate than said coagulating liquid; subjecting said fiber to a subsequent-wash treatment with an aqueous liquid which is substantially free from ethylene carbonate; continuously diverting at least a portion of the effluent resulting from said subsequent-wash treatment and incorporating the same in the liquid used in said hot-stretching treatment so as to assist the maintenance of said hot-stretching liquid at said concentration; drying said washed fiber.

7. A method according to claim 6 wherein the stretched fiber resulting from said hot-stretching treatment contains less than about 175% by weight of ethylene carbonate and the fiber is stretched to a total length at least about 300% of the original length as withdrawn from the coagulating liquid.

8. In the method of making acrylonitrile polymer fibers by extruding into a coagulating liquid comprising water and between about 10% and 50% by weight of ethylene carbonate, a spinning solution comprising ethylene carbonate, water in an amount between about 2.5% and 18.5% by weight, and a polymer of acrylonitrile contain-

ing in the polymer molecule at least about 80% by weight of acrylonitrile, performing in a continuous manner and on a continuous length of fiber the steps comprising, withdrawing the resulting fiber from said coagulating liquid; orienting said fiber by stretching it to a length at least about 150% of its original length at a temperature below about 65° C.; stretching said fiber to a length at least about 150% of its length while in the presence of an aqueous liquid maintained at a temperature above about 95° C., said hot aqueous liquid comprising water and between about 1% and 6% by weight of ethylene carbonate; withdrawing said stretched fiber from said hot-stretching liquid; subjecting said fiber to an intermediate-wash treatment with an aqueous liquid comprising water and ethylene carbonate while said fiber is being conducted over at least one rotating thread-supporting device, said intermediate-wash liquid having a lower concentration of ethylene carbonate than said coagulating liquid but greater than said hot-stretching liquid, said intermediate-wash liquid being prepared by continuously incorporating at least a portion of the effluent resulting from said hot-stretching treatment; continuously diverting at least a portion of the effluent from said intermediate-wash treatment and continuously fortifying said coagulating liquid therewith so as to maintain said coagulating liquid at said concentration, said diverted liquid containing less ethylene carbonate than said coagulating liquid; subjecting said fiber, while it is being conducted over at least one rotating thread-supporting device, to a subsequent-wash treatment with an aqueous liquid which is substantially free from ethylene carbonate; continuously diverting at least a portion of the effluent resulting from said subsequent-wash treatment and incorporating the same in the liquid used in said hot-stretching treatment so as to assist the maintenance of said hot-stretching liquid at said concentration; drying said washed fiber.

9. A method according to claim 8 in which the fiber, which is conducted over the rotating thread-supporting devices for the performance of the intermediate and subsequent-wash treatments, is in the form of a helix; and in which the fiber is washed substantially free of ethylene carbonate while being subjected to the subsequent-wash treatment.

10. A method according to claim 8 wherein the fiber is washed to no more than 3% by weight of ethylene carbonate after being subjected to the subsequent-wash treatment.

11. A method according to claim 6 in which the effluent from the intermediate-wash treatment, which is being diverted for use in fortifying the aqueous coagulating liquid, contains ethylene carbonate in a concentration of at least about 5% by weight less than the concentration of ethylene carbonate in the coagulating liquid.

12. A method according to claim 6 in which the effluent from the subsequent-wash treatment, which is being diverted for use in the hot-stretching treatment, contains less than about 3% by weight of ethylene carbonate; and in which the effluent from the intermediate-wash treatment, which is being diverted for use in fortifying the aqueous coagulating liquid, contains ethylene carbonate in a concentration at least about 5% by weight less than the concentration of ethylene carbonate in the coagulating liquid.

13. A method according to claim 8 in which the effluent from the subsequent-wash treatment, which is being diverted for use in the hot-stretching treatment, contains less than about 3% by weight of ethylene carbonate; and in which the effluent from the intermediate-wash treatment, which is being diverted for use in fortifying the aqueous coagulating liquid, contains ethylene carbonate in a concentration at least about 5% by weight less than the concentration of ethylene carbonate in the coagulating liquid.

14. A method according to claim 6 in which substantially all of the water present in all of the aqueous treat-

ment steps recited from the coagulating step to the subsequent-wash treatment, with the exception of the water introduced by the spinning solution, is introduced at the subsequent-wash treatment step.

15. A method according to claim 8 in which substantially all of the water present in all of the aqueous treatment steps recited from the coagulating step to the subsequent-wash treatment, with the exception of the water introduced by the spinning solution, is introduced at the subsequent-wash treatment step.

16. A method according to claim 3 wherein the portion of the effluent from the intermediate-wash treatment, which is continuously diverted to fortify the coagulating liquid, contains no more than about eight and one-half parts by weight of water for each part by weight of spinning solution extruded.

17. A method according to claim 8 wherein the portion of the effluent from the intermediate-wash treatment, which is continuously diverted to fortify the coagulating liquid, contains no more than about eight and one-half parts by weight of water for each part by weight of spinning solution extruded.

18. A method according to claim 17 wherein said portion of the effluent from the intermediate-wash treatment contains at least about five parts by weight of water 25 for each part by weight of said acrylonitrile polymer solids extruded into said coagulating liquid.

19. In the method of making acrylonitrile polymer fibers having a denier greater than about 2,000 by extruding into a coagulating liquid comprising water and between about 20% and 38% by weight of ethylene carbonate maintained at a temperature between about 40° and 90° C., a spinning solution maintained at a temperature between about 50° and 75° C. comprising ethylene carbonate, water in an amount between about 10% and 15% by weight, and about 12% and 18% by weight of a polymer of acrylonitrile containing in the polymer molecule at least about 80% by weight of acrylonitrile, performing in a continuous manner and on a continuous length of fiber the steps comprising, withdrawing the resulting fiber from said coagulating liquid; orienting said fiber by stretching it to a length at least about 150% of its original length at a temperature below about 100° C.; stretching said fiber to a length at least about 150% of its length while in the presence of an aqueous liquid maintained at a temperature above about 95° C., said hot liquid comprising water and between about 1% and 6% by weight of ethylene carbonate; withdrawing said stretched fiber from said hot-stretching liquid; subjecting said fiber to an intermediate-wash treatment with an aqueous liquid comprising water and ethylene carbonate, said intermediate-wash liquid having a concentration of ethylene carbonate greater than said hot-stretching liquid and at least about 5% by weight less than the concentration of ethylene carbonate in said coagulating liquid, said intermediate-wash liquid being prepared by continuously incorporating therein the effluent resulting from said hot-stretching treatment; continuously diverting the effluent resulting from said intermediate-wash treatment and continuously fortifying said coagulating liquid therewith so as to maintain the coagulating liquid at said concentration; subjecting each part by dry weight of said fiber to a subsequent-wash treatment with between about eight and about twenty-seven parts by weight of water which is substantially free from ethylene carbonate thereby washing said fiber to less than about 3% by weight of residual ethylene carbonate; continuously diverting the effluent resulting from said subsequent-wash treatment and incorporating the same in the liquid used in said hot-stretching treatment; continuously recovering purified ethylene carbonate from the effluent from said coagulating liquid; preparing at least a portion of said spinning solution with said

5 10 15 20 25 30 35 40 45 50 55 60 65 70

recovered ethylene carbonate; drying said washed fiber.

20. A method according to claim 19 in which the fiber is stretched while being washed with the hot aqueous liquid for not more than one second and in which the fiber is washed to less than about 0.5% by weight of residual ethylene carbonate after being subjected to the subsequent-wash treatment.

21. In the method of making acrylonitrile polymer fibers having a denier greater than about 2,000 by extruding into a coagulating liquid comprising water and between about 20% and 38% by weight of ethylene carbonate maintained at a temperature between about 40° and 90° C., a spinning solution maintained at a temperature between about 50° and 75° C. comprising ethylene carbonate, water in an amount between about 10% and 15% by weight, and about 12% and 18% by weight of a polymer of acrylonitrile containing in the polymer molecule at least about 80% by weight of acrylonitrile, performing in a continuous manner and on a continuous length of fiber the steps comprising, withdrawing the resulting fiber from said coagulating liquid; orienting said fiber by stretching it to a length at least about 150% of its original length at a temperature below about 100° C.; stretching said fiber again to a length at least about 150% of its length while in the presence of an aqueous liquid maintained at a temperature above about 95° C., said hot aqueous liquid comprising water and between about 1% and 6% by weight of ethylene carbonate; withdrawing said stretched fiber from said hot-stretching liquid; subjecting said fiber to an intermediate-wash treatment with an aqueous liquid maintained at a temperature no greater than about 60° C. comprising water and ethylene carbonate, said intermediate-wash liquid having a concentration of ethylene carbonate greater than said hot-stretching liquid and at least about 5% by weight less than the concentration of ethylene carbonate in said coagulating liquid, said intermediate-wash liquid being prepared by continuously incorporating therein the effluent resulting from said hot-stretching treatment after rapidly cooling said effluent to the temperature of the intermediate-wash; continuously diverting the effluent resulting from said intermediate-wash treatment and continuously fortifying said coagulating liquid therewith so as to maintain the coagulating liquid at said concentration; subjecting each part by dry weight of said fiber to a subsequent-wash treatment with between about eight and about twenty-seven parts by weight of water which is substantially free from ethylene carbonate maintained at a temperature no greater than about 60° C. thereby washing said fiber to less than about 3% by weight of residual ethylene carbonate; continuously diverting the effluent resulting from said subsequent-wash treatment and rapidly heating said effluent to a temperature above about 95° C. and incorporating the same in the liquid used in said hot-stretching treatment; continuously recovering purified ethylene carbonate from the effluent from said coagulating liquid; preparing at least a portion of said spinning solution with said recovered ethylene carbonate; drying said washed fiber.

22. A method according to claim 21 in which the fiber is stretched while being subjected to the hot-stretch liquid for not more than two and one-half seconds and in which the fiber is washed to less than about 0.5% by weight of ethylene carbonate after being subjected to the subsequent-wash treatment.

#### References Cited in the file of this patent

#### UNITED STATES PATENTS

|    |           |          |               |
|----|-----------|----------|---------------|
| 70 | 2,530,962 | Hare     | Nov. 21, 1950 |
|    | 2,570,257 | McFarren | Oct. 9, 1951  |
|    | 2,577,763 | Hoxic    | Dec. 11, 1951 |